

## 1

2,704,745

STABILIZED EXTREME PRESSURE LUBRICANT  
 Harry L. Kopp, Alexandria, Va., and Leo W. Manley,  
 Woodbury, N. J., assignors to Socony-Vacuum Oil  
 Company, Incorporated, a corporation of New York  
 No Drawing. Application February 1, 1954,  
 Serial No. 407,574

7 Claims. (Cl. 252—37.2)

This invention relates to the art of lubrication and is particularly concerned with lubricants suitable for use under abnormally high pressures, such as are encountered between engaged surfaces in various types of modern industrial machinery, such as the worm gears and the like. The so-called "extreme pressure" lubricants with which this invention is concerned comprise a mineral lubricating oil having dissolved or dispersed therein one or more chemical agents which will provide between the engaged surfaces a lubricating film capable of withstanding high pressures. The invention is specifically concerned with extreme pressure lubricants of this type which possess high oxidation stability.

It was recognized in the past that the presence of sulfur or sulfur-containing compounds in a lubricating oil enhanced the load-carrying ability of the oil. Thus, for example, Smackover Black Oil, an unrefined residuum stock of high-sulfur content, was known to possess good extreme pressure properties. Later, it was found that the load-carrying ability of such high-sulfur oils could be greatly improved by the incorporation therein of certain heavy metal soaps. Lead naphthenate, for example, was found to be outstandingly effective in this respect. A serious drawback, however, with respect to the use of lead naphthenate was that it reduced the oxidation stability of the oil. The degree of oxidation stability is manifested by the rate of increase in viscosity of the oil in use, an oil which is highly unstable becoming quite viscous in a relatively short time.

It was later found that the oxidation stability of compositions containing lead naphthenate could be greatly improved without diminishing their extreme pressure ability by utilizing a synthetic sulfur compound, such as dibenzyl disulfide, as a source of sulfur along with a relatively stable base oil rather than using relatively unstable high sulfur content base oils, *per se*. Thus, the oils used in these compositions were oils which had been refined to remove unstable components thereof. A considerable variety of organic sulfur-containing compounds have been utilized in combination with lead naphthenate in oils of this type. For example, a typical chemical extreme pressure composition employs dibenzyl disulfide and lead naphthenate in a Pennsylvania cylinder type oil.

We have now found that the oxidation stability of extreme pressure compositions of the last-defined type can be improved even further, and without impairment of their extreme pressure character, by utilizing as the synthetic extreme pressure agent an organic compound containing both sulfur and nitrogen, rather than a compound containing sulfur alone.

Only certain sulfur- and nitrogen-containing organic compounds, however, are suitable for use in the invention, since only these meet all the requirements necessary for use as an extreme pressure agent in a mineral oil type lubricant. Thus, such additives must possess the following characteristics: (1) adequate oil solubility, (2) adequate load-carrying ability, (3) relative inactivity towards copper and (4) adequate oxidation inhibition. The sulfur- and nitrogen-containing compounds which have been found to meet all of these requirements are: 2-benzothiazyl N-N diethyl thio carbamyl sulfide, 2-benzothiazyl N-N dibutyl thio carbamyl sulfide, oxypentamethylene thio carbamyl diethyl thio carbamyl sulfide, bis-4-methylbenzothiazyl disulfide, benzothiazyl-N-butyl disulfide and benzothiazyl-tert-butyl disulfide.

It is, therefore, the object of this invention to provide extreme pressure lubricating oil compositions of superior oxidation stability, said compositions containing in com-

## 2

bination one of the aforementioned sulfur- and nitrogen-containing compounds and lead naphthenate. Other and further objects will become apparent hereinafter.

As previously indicated, the base oils contemplated for use in the compositions of the invention are oils which have been refined to remove unstable components thereof, such as by solvent-refining. The oil need not be of any particular source or type and may range in viscosity from as low as 100 seconds S. U. V. at 100° F. to as high as 500 seconds at 210° F., depending upon the application for which the lubricant is intended. The invention, therefore, provides highly stable extreme pressure lubricating compositions comprising a refined mineral lubricating oil and minor proportions of one of the aforementioned sulfur- and nitrogen-containing organic compounds and lead naphthenate.

The uniqueness of the several sulfur- and nitrogen-containing organic compounds of the invention as extreme pressure agents as compared to organic sulfur- and nitrogen-containing compounds in general is shown by the data given in Table I. This table lists a number of other sulfur- and nitrogen-containing organic compounds which were tested and found not suitable for failure to meet one or more of the requirements necessary for extreme pressure oil additives as mentioned hereinabove. The procedures utilized in testing these compounds were as follows:

1. The copper strip corrosion test procedure was that of A. S. T. M. Method D130-50T (A. S. T. M. Standards on Petroleum Products and Lubricants, November 1952, pages 81-84).

2. The Timken test was conducted according to CRC Method L-18-545 (CRC Handbook, 1946 edition, pages 462-466).

3. The oil solubility test was conducted by preparing hand blends of the compounds in light mineral oil and visibly observing the clarity of the blends.

4. The oxidation test simulates oxidation which occurs in industrial equipment, such as gear sets in which the oil is churned and intimately mixed with air. The test oil is subjected to a temperature of 250° F. and stirred with a paddle made of 2" x 2" copper and steel plates bolted together. The paddle is immersed in the oil and turned at a speed of 205±5 R. P. M., thereby mixing air into the oil. Viscosity measurements are taken on the oil before the test, periodically during the test and at fourteen days, the end of the test. Percent increase in viscosity is determined.

The base oil used in all tests was a Pennsylvania cylinder oil having a Saybolt Universal viscosity of 150 seconds at 210° F.

Table I

|    | Compound                                                        | Deficiency                         |
|----|-----------------------------------------------------------------|------------------------------------|
| 55 | Benzothiazyl disulfide.....                                     | Poor oil-solubility.               |
|    | 85% dimethyl-2-mercaptothiazole.....                            | Do.                                |
|    | 15% 4-ethyl-2-mercaptothiazole.....                             | Inadequate load-carrying capacity. |
| 60 | 2,4 dinitrophenylthiobenzothiazole.....                         | Do.                                |
|    | 2-dodecylthiobenzothiazole.....                                 | Do.                                |
|    | Bis-2-benzothiazyl monosulfide.....                             | Breaks down to insoluble compound. |
|    | N-cyclohexyl 2-benzothiazyl sulfonamide.....                    | Inadequate load-carrying capacity. |
| 65 | 2-benzothiazyl thiol benzoate.....                              | Do.                                |
|    | n-octyl-N,N-diethylthionourethan.....                           | Corrosive to copper.               |
|    | Phenyl-N,N-diethylthionourethan.....                            | Poor oil-solubility.               |
|    | Pentachlorophenyl-N,N-diethylthionourethan.....                 | Corrosive to copper.               |
|    | 2,4-dichlorophenyl-N,N-diethylthionone carbamate.....           | Inadequate load-carrying capacity. |
| 70 | N,N-diethyl-N',N-diphenyl thiourea.....                         | Do.                                |
|    | N,N'-diphenyl-N-diethyl thiocarbamyl-p-phenylene diamine.....   | Poor oil-solubility.               |
|    | Pentamethylene thiocarbamyl diethyl thio carbamyl sulfide.....  | Corrosive to copper.               |
|    | Unsym.-diethyl di(2-ethoxy ethyl) thiurane sulfide.....         | Do.                                |
|    | 2-benzothiazole-N-cyclopentamethylene thiocarbamyl sulfide..... | Poor oil-solubility.               |
|    | 1,3,4-thiadiazolyl-2,5-bis(diethyl dithiocarbamate).            | Do.                                |
| 75 | 3-phenyl-2-thiono 4-1,3,4-thiadiazolinyl dithiocarbamate.       | Do.                                |
| 80 |                                                                 |                                    |

## 3

In contrast to the sulfur-nitrogen compounds shown in Table I, the several sulfur-nitrogen compounds contemplated by the invention all proved entirely satisfactory from the standpoint of their oil-solubility and copper corrosion characteristics. In addition, these compounds provided extreme pressure lubricants of outstanding stability toward oxidation, as shown by the data in Table II. This table shows the results of extreme pressure and oxidation tests made on typical compositions prepared using the several sulfur-nitrogen compounds of the invention and on a typical lubricant of the commercial type employing dibenzyl disulfide. It will be seen that in all cases the compositions contemplated by the invention showed a marked superiority to the commercial lubricant in oxidation stability; and, in all cases, except one, a marked improvement in load-carrying capacity. In no case was the load-carrying capacity below that obtained with the commercial lubricant. The Timken and oxidation test procedures in all cases were the same as those utilized in testing the compounds shown in Table I. The base oil was also the same as that used in testing the compounds listed in Table I.

Table II

| Product Blended in Oil                                             | Timken O. K. Load, Lbs. | Oxidation Test (14 Days), Vis. Increase @ 210° F., Percent |
|--------------------------------------------------------------------|-------------------------|------------------------------------------------------------|
| None                                                               | 10                      | 24                                                         |
| 5% Lead Naphthenate                                                | 20                      | 68                                                         |
| 5% Dibenzyl Disulfide                                              | 35                      | 69                                                         |
| 5% Lead Naphthenate                                                | 50                      | 27                                                         |
| 0.25% 2-Benzothiazyl N-N Diethyl Thio Carbamyl Sulfide             | 35                      | 26                                                         |
| 5% Lead Naphthenate                                                | 50                      | 58                                                         |
| 0.5% 2-Benzothiazyl N-N Dibutyl Thio Carbamyl Sulfide              | 45                      | 38                                                         |
| 5% Lead Naphthenate                                                | 45                      | 35                                                         |
| 0.25% Oxpentamethylene Thio Carbamyl Diethyl Thio Carbamyl Sulfide | 45                      | 35                                                         |
| 5% Lead Naphthenate                                                | 45                      | 35                                                         |
| 0.5% Bis-4-Methylbenzothiazyl Disulfide                            | 45                      | 35                                                         |
| 5% Lead Naphthenate                                                | 45                      | 35                                                         |
| 0.25% Benzothiazyl-N-Butyl Disulfide                               | 45                      | 35                                                         |
| 5% Lead Naphthenate                                                | 45                      | 35                                                         |
| 0.25% Benzothiazyl-Tert-Butyl Disulfide                            | 45                      | 35                                                         |
| 5% Lead Naphthenate                                                | 45                      | 35                                                         |

All of the sulfur- and nitrogen-containing compounds utilized in the invention were obtained from chemical manufacturers, principally Sharples Chemicals, Inc., Wyandotte, Michigan, and Monsanto Chemical Company, St. Louis, Missouri. They may be further identified by their chemical formulae as follows:

2-benzothiazyl N-N diethyl thio carbamyl sulfide



2-benzothiazyl N-N dibutyl thio carbamyl sulfide



Oxpentamethylene thio carbamyl diethyl thio carbamyl sulfide



Bis-4-methylbenzothiazyl disulfide



## 4

Benzothiazyl-N-butyl disulfide



Benzothiazyl-t-butyl disulfide



- 15 Since these compounds are known to the art and may be prepared by a number of different methods, specific details with respect to their preparation will not be given here. Briefly, however, 2-benzothiazyl N-N diethyl thio carbamyl sulfide and 2-benzothiazyl N-N dibutyl thio carbamyl sulfide may be made by reaction of sodium mercaptobenzothiazole with N-diethyl thiono carbamyl chloride and N-dibutyl thiono carbamyl chloride, respectively. Bis-4-methylbenzothiazyl disulfide may be prepared by oxidation in an aqueous solution of sodium mercaptobenzothiazole using chlorine as the oxidizing agent. Benzothiazyl-N-butyl and benzothiazyl tertiary butyl disulfide may be made by reaction of N-butyl disulfide and tertiary butyl disulfide, respectively, with bis-benzothiazyl disulfide in the presence of sodium sulfide and ethyl alcohol at 100° C., and oxypentamethylene thio carbamyl diethyl thio carbamyl sulfide may be prepared by reaction of morpholine with diethyl amine and carbon disulfide.

Although the specific compositions shown herein, for purposes of comparison, all contain 5 weight per cent lead naphthenate and either 0.25 or 0.5 weight per cent of the sulfur-nitrogen compound, the amount of each of these additives can be varied within reasonable limits, depending upon the particular application for which the lubricant is designed. Thus, the amount of lead naphthenate which may be used ranges from about 1 to about 20 weight per cent, while the amount of the sulfur-nitrogen compound may be from about 0.1 to about 3.0 weight per cent.

35 45 Additional additives, designed to impart various other lubricating characteristics to the compositions of this invention, such as pour depressants, viscosity index improvers, etc., may be used therein, if desired.

Having now fully described the invention, what is

50 claimed as new and patentable is:

1. A lubricant composition comprising a major proportion of a refined mineral lubricating oil and (1) from about 0.1% to about 3.0% by weight of a sulfur- and nitrogen-containing organic compound selected from the group consisting of 2-benzothiazyl N-N diethyl thio carbamyl sulfide, 2-benzothiazyl N-N dibutyl thio carbamyl sulfide, oxypentamethylene thio carbamyl diethyl thio carbamyl sulfide, bis-4-methylbenzothiazyl disulfide, benzothiazyl-N-butyl disulfide and benzothiazyl-tert-butyl disulfide and (2) from about 1% to about 20% by weight of lead naphthenate.

55 60 65 2. A lubricant composition comprising a major proportion of a refined mineral lubricating oil and (1) from about 0.1% to about 3.0% by weight of 2-benzothiazyl N-N diethyl thio carbamyl sulfide and (2) from about 1% to about 20% by weight of lead naphthenate.

3. A lubricant composition comprising a major proportion of a refined mineral lubricating oil and (1) from about 0.1% to about 3.0% by weight of 2-benzothiazyl N-N dibutyl thio carbamyl sulfide and (2) from about 1% to about 20% by weight of lead naphthenate.

70 75 80 4. A lubricant composition comprising a major proportion of a refined mineral lubricating oil and (1) from about 0.1% to about 3.0% by weight of oxypentamethylene thio carbamyl diethyl thio carbamyl sulfide and (2) from about 1% to about 20% by weight of lead naphthenate.

5. A lubricant composition comprising a major proportion of a refined mineral lubricating oil and (1) from about 0.1% to about 3.0% by weight of bis-4-methylbenzothiazyl disulfide and (2) from about 1% to about 20% by weight of lead naphthenate.

85 6. A lubricant composition comprising a major proportion of a refined mineral lubricating oil and (1) from about 0.1% to about 3.0% by weight of benzothiazyl-

N-butyl disulfide and (2) from about 1% to about 20% by weight of lead naphthenate.

7. A lubricant composition comprising a major proportion of a refined mineral lubricating oil and (1) from about 0.1% to about 3.0% by weight of benzothiazyl-  
tert-butyl disulfide and (2) from about 1% to about 20% by weight of lead naphthenate.

## References Cited in the file of this patent

## UNITED STATES PATENTS

|   |           |                |               |
|---|-----------|----------------|---------------|
| 5 | 2,154,097 | Loane          | Apr. 11, 1939 |
|   | 2,218,283 | Fuller         | Oct. 15, 1940 |
|   | 2,237,526 | Humphreys      | Apr. 8, 1941  |
|   | 2,367,355 | Kaufman et al. | Jan. 16, 1945 |